

June 11, 1940.

B. R. F. KJELLGREN ET AL

2,204,221

PROCESS FOR PRODUCING BERYLLIUM

Filed Aug. 18, 1939



FIG. 1.



FIG. 2.

INVENTORS:  
Bengt R. F. Kjellgren  
Charles B. Sawyer  
BY Ray A. Ehr  
ATTORNEY

## UNITED STATES PATENT OFFICE

2,204,221

## PROCESS FOR PRODUCING BERYLLIUM

Bengt R. F. Kjellgren, Rocky River, and Charles B. Sawyer, Cleveland Heights, Ohio, assignors to The Brush Beryllium Company, Cleveland, Ohio, a corporation of Ohio

Application September 18, 1939, Serial No. 295,474

4 Claims. (Cl. 75—84)

This invention relates to an improved process for the recovery of beryllium wherein beryllium oxide is reduced with the aid of carbonaceous reducing agents and metallic beryllium is evolved in a vapor state and relates particularly to a process in which the distilled beryllium is recovered in a highly pure state.

Attempts have heretofore been made to produce metallic beryllium by distillation in connection with the reduction of beryllium oxide with carbon, for instance by heating a mixture of beryllium oxide and carbon in an electric furnace to a temperature of the order of 2000° C. But the attempts made in this direction have not led to any useful results because the rate of reaction and evolution of beryllium under such conditions has been too slow for commercial use. Attempts have been made to increase the rate of reaction by operating in a vacuum or by flowing a strong current of hydrogen through the charge, but these expedients have not improved the rate of reaction to any marked extent.

It is an object of this invention to provide a distillation process for the recovery of beryllium which is characterized by a much higher rate of reaction under commercial conditions than has heretofore been obtained.

A further object of the invention is to provide a process of the character last referred to adapted to produce metallic beryllium of a high degree of purity.

Our improved process is based upon the discovery that the rate of reaction between beryllium oxide and carbon is markedly affected by the degree of purity of the oxide. In our process of producing alloys containing beryllium set forth in our application Serial No. 89,362, filed July 7, 1936, which has matured into Patent No. 2,176,906, we have made use of this discovery and in our present process the discovery is taken advantage of for the production of metallic beryllium by heating a mixture of suitably pure beryllium oxide and carbon, preferably in stoichiometric proportions, to a temperature at which the reduced beryllium is disengaged in the form of vapor. A temperature of at least 1900° C. is necessary for this. Reduced pressure or vacuum may be resorted to, but preferably a stream of hydrogen, or other inert gas such as helium, is passed through the reaction zone. The stream of gas sweeps the beryllium vapor from the reaction zone and carries it into contact with suitable condensing means where it is cooled suddenly and thereby substantially prevented from being reoxidized by the carbon monoxide generated by

the reducing reaction and carried out of the reaction zone with the beryllium vapor. Metallic beryllium is recovered in a pure condition from the condensing device, while any entrained beryllium which escapes from the condensing means may be recovered from the carbon monoxide and hydrogen gases issuing therefrom by passing the gas through filters or centrifugal separators. If desired the hydrogen component of the gas mixture may also be recovered and recycled so as to operate the process with maximum economy.

As indicated, a stream of inert gas such as hydrogen or helium is used in the process since through its use the beryllium vapor may be swept out of the reaction zone as rapidly as it is formed, the vapor pressure of beryllium being thereby kept at such a low value that the maximum rate of reaction between the beryllium oxide and carbon is favored. Furthermore, as indicated above, the stream of gas aids in condensing the beryllium vapor without the latter being reoxidized.

As has been indicated, the present invention rests essentially upon the discovery that when high purity beryllium oxide is substituted for less pure oxide, the rate of production of beryllium vapor, and hence of beryllium, can be greatly increased, the increase in fact being far out of proportion to any change which might be expected from the slight change in purity of the oxide. Without wishing to be limited by the theory expressed, we believe this result is due in part to the fact that the higher purity oxide is less dense and exposes more surface to the reducing action of the carbon, and in part to the fact that by eliminating impurities such as calcium oxide, silica, alumina, and like fluxes, sintering or melting of the charge is avoided with the consequent result that the initially large area exposed by the pure oxide is not lessened when the charge is heated to the very high temperatures which must be employed, and furthermore is not diminished appreciably during any of the time that the beryllium oxide is being reduced by the carbon. A high rate of reaction may therefore be attained and maintained. Moreover, in our process the oxide and carbon mixture preferably is heated in a loose state and the beryllium vapors disengaged by the reducing reaction are evolved in a loose, highly porous charge from which they may readily escape so as to be swept out by the current of hydrogen. The beryllium vapors accordingly do not have opportunity to accumulate within the charge to such an extent that their

concentration therein approaches the limit at which the reaction is suppressed.

The following experimental results will illustrate the magnitude of the improvement which 5 results when high purity oxide is substituted for lower purity material. In these experiments charges were prepared and treated in pairs, the charges of each pair being as nearly identical as possible except for their purity, both charges 10 containing the same weight of oxide intimately mixed with the same proportions of carbonaceous reducing agent. One charge of each pair was made up with beryllium oxide containing 0.3% calcium oxide and somewhat less than 99.7% 15 beryllium oxide, while the other charge was made up with beryllium oxide containing impurities totalling less than 0.1%, the iron oxide, calcium oxide, silica and alumina each mounting to less than 0.02%. Both charges were heated 20 individually in an induction furnace at the same rate and for the same lengths of time and were subjected to the same rate of hydrogen flow. In short, they were treated in identical manners, so that the purity of the oxide would be the only 25 variable effecting a difference in the rate of evolution of beryllium from the charges. When the charges were treated in this way it was found that the rate of evolution of beryllium from the high purity sample was about double the rate 30 of evolution from the sample containing 0.3% calcium oxide, example values of the rates being 24.5% per hour and 12.4% respectively. It will be appreciated that an increase of this magnitude in the rate of production permits extensive economies 35 in operating costs since the time required to produce a unit of beryllium is reduced to about half of the corresponding time required when the less pure material is used. The improvement greatly enhances the commercial value 40 of the distillation method of producing beryllium.

In practicing the present invention beryllium oxide of a suitable degree of purity can be selected, as hereinafter described, from the products now commercially available. Carbon is preferably 45 used as reducing agent although beryllium carbide is also suitable for use and can be used either alone or in combination with carbon. Such reducing agents as calcium carbide, calcium silicide, metallic silicon, or silicon alloys should be avoided 50 since they produce metallic oxides and/or silica which remain in the furnace and flux the charge, thus creating the disadvantages which are to be avoided by the use of the high purity material. For the same reason, carbonaceous reducing agents which contain large amounts of 55 metallic oxides as impurities should be avoided. Graphite and resistor carbon are generally of moderate purity and are suitable for use as reducing agents. The reducing agent should, of course, be intimately mixed with the beryllium oxide in order to obtain the most favorable conditions for efficient reduction, and the charge should preferably be introduced into the reaction 60 zone in a loose, pulverulent condition, since under such conditions the stream of hydrogen may be used most effectively in maintaining a low vapor pressure of beryllium within the charge. The temperatures employed to effect reduction are of the same order as those heretofore proposed in 65 connection with the use of impure starting materials, being generally above 1900° C. and preferably around 2100° C. At these temperatures various hydrocarbons, of which acetylene is an example, are formed through reaction of the 70 hydrogen with the carbonaceous reducing agent.

Being gases at the high temperatures employed, and having strong reducing properties, these materials aid in reducing the beryllium oxide.

In the operation of the process, use may be made of various forms and kinds of apparatus 5 such as those heretofore used or proposed for use in the production of beryllium by distillation or for analogous purposes. Thus, for example, heating of the charge may be accomplished by a furnace wherein the charge is heated by high 10 frequency induction, a carbon arc, or electrical resistance or wherein the charge forms one or both electrodes of an electric arc.

For the purpose of further explaining and 15 illustrating the invention a suitable specific procedure will be described with reference to the accompanying drawing.

In the drawing,

Fig. 1 is a flow sheet indicating the steps of a preferred procedure in carrying out the inven- 20

Fig. 2 is a sectional view of apparatus which may be used in selecting a suitably pure beryllium oxide by determination of its apparent density.

In describing the procedure indicated in Fig. 1 25 of the drawing, reference will first be made to the selection of the beryllium oxide. Generally speaking, beryllium oxide which is not sufficiently pure to resist sintering at a temperature of 1600° C. is not suitable for the present process, and 30 preferably the oxide should be pure enough to resist substantial sintering at the temperature of the reduction reaction as carried out in the 35 practice of the process. The troublesome impurities most frequently encountered in the beryllium oxide are calcium oxide and silicon-oxide, though there may be others. Undecomposed sulfate may also cause trouble.

Since the density of beryllium oxide increases 40 with increase in the amount of impurities, a very good practical test for adequate purity of the beryllium oxide is its apparent density. In order 45 that the term "apparent density" as herein used may have a definite meaning, it is to be understood that the determination of such density is carried out in accordance with the following procedure. First, the sample of oxide used for the determination is to be heated, for the first time, for a period of ten minutes at a temperature of 1600° C. in an atmosphere not more reducing 50 than that of hydrogen. In carrying out the heat treatment, the beryllium oxide is passed through an 80 mesh screen and allowed to fall lightly into a refractory boat which is to hold it during the heating operation. In Fig. 2 we have shown apparatus 55 to be used in determining the apparent density of the heat-treated material. The apparatus consists of a sieve 1 comprising a frame or side wall 2 and screen 3 having 20 openings per inch, the wire of the screen having a diameter of 0.0172 inch and the individual screen openings having an area of 0.0328 square inch. The sieve is supported as shown in a large glass funnel 4 which in turn is suitably supported above a weighing bottle or cup 5. The full size dimensions 60 of each piece of the apparatus are indicated in the figure.

In making the apparent density determination after heating the sample to 1600° C. as above described, an amount of the beryllium oxide sufficient 70 to slightly more than fill the weighing bottle is placed upon the screen 3 and brushed through so as to fall through the funnel, without packing, into the weighing bottle the volume of which, at a height level with its top, is known. The small 75

excess of beryllium oxide is scraped off (without packing) to leave the material even with the bottle top. The weight of the oxide in the weighing bottle is then determined and the apparent density calculated from the known volume and the determined weight.

For the best operation of the process the apparent density of the beryllium oxide, determined as above described, should be less than 0.4. If it 10 is greater than 0.5 the operation is unsatisfactory since considerable quantities of sintered oxide are formed, causing loss of exposed oxide surface and interfering with speedy reduction.

As a suitable procedure in practicing the 15 method represented by Fig. 1 of the drawing, high purity oxide having an apparent density less than 0.5 and preferably less than 0.4 is intimately mixed with a stoichiometric amount of finely ground graphite, resistor carbon, 20 beryllium carbide, or mixtures thereof, and the mixture is introduced in a loose condition into the reaction chamber of a suitable electric furnace and through which a current of preheated hydrogen flows. Preferably the charge is heated 25 rapidly to a temperature above 1900° C., at which temperature the beryllium oxide is reduced by the reducing agent and yields vaporous beryllium and carbon monoxide. By reason of the stream of hydrogen flowing through the reaction zone, 30 the carbon monoxide is diluted as it and the beryllium vapor are swept out of the reaction zone. The gaseous stream may be caused to impinge on extensive cooled surfaces or otherwise treated to condense the beryllium vapor without 35 permitting the carbon monoxide to act upon it to reoxidize it to beryllium oxide. Methods and apparatus for effecting this type of condensation are, as previously indicated, well known in the art and form no part of the present invention. 40 Accordingly the step is merely indicated diagrammatically in the flow sheet and need not be discussed in further detail. As indicated above, some beryllium may not be condensed in the condensing system and is carried along in the gas 45 stream issuing therefrom. This beryllium is generally in the form of a fine powder the particles of which are partially or fully coated with beryllium oxide and/or beryllium carbide. This powder may be separated from the gases in any 50 suitable way, many of which are well known in the art. The gas stream may then be treated in known manner to recover the hydrogen which it contains, the recovered hydrogen being recycled through the process.

55 It will thus be seen that beryllium is recovered in at least two different forms, the material recovered from the condensing system being in a highly pure state since it is uncontaminated with

any of the usual impurities which may occur in beryllium oxide and which would be vaporized and condensed along with the beryllium. The other beryllium product, consisting of a fine powder containing a minor amount of metallic 5 beryllium and a major amount of beryllium oxide or carbide, may be mixed with graphite and recycled by including it in subsequent charges which are introduced into the distillation furnace.

10 In the following claims, the term "carbonaceous reducing agent" is used to mean carbon-containing material capable of reducing beryllium oxide at the temperatures employed, and including beryllium carbide, hydrocarbons, or some form 15 of carbon, or mixtures of these materials.

Having now explained our invention, what we claim is:

1. In a process for recovering beryllium by thermal reduction wherein beryllium oxide is decomposed by reaction with carbonaceous reducing agent at temperatures above about 1900° C. and wherein the reduced beryllium is removed from the reaction zone in vapor form and subsequently condensed, the step of using high purity 25 beryllium oxide having an apparent density of less than 0.5.

2. In a process for recovering beryllium by thermal reduction wherein beryllium oxide is decomposed by reaction with carbonaceous reducing agent at temperatures around 2100° C., and wherein the reduced beryllium is removed from the reaction zone in vapor form and subsequently condensed, the step of using high purity 35 beryllium oxide having an apparent density of less than 0.4.

3. In a process for producing beryllium by thermal reduction of its oxide wherein beryllium oxide is decomposed by reaction with carbonaceous reducing agent at temperatures above 40 about 1900° C., and wherein the reduced beryllium is removed from the reaction zone in vapor form by a current of hydrogen and is subsequently condensed and recovered as metallic beryllium, the step of using high purity beryllium 45 oxide having an apparent density of less than 0.5.

4. In a process for producing beryllium by thermal reduction of its oxide wherein beryllium oxide is decomposed by reaction with carbonaceous reducing agent at temperatures around 2100° C., 50 and wherein the reduced beryllium is removed from the reaction zone in vapor form by a current of hydrogen and is subsequently condensed and recovered as metallic beryllium, the step of using high purity beryllium oxide having an apparent density of less than 0.4.

BENGT R. F. KJELLGREN.  
CHARLES B. SAWYER.